

## UNITED STATES PATENT OFFICE

STERLING HENRY DIGGS AND FRANK S. CAMPBELL, OF CASPER, WYOMING, ASSIGNEES  
TO STANDARD OIL COMPANY, OF WHITING, INDIANA, A CORPORATION OF INDIANA

## LEAD COMPOUND

No Drawing.

Application filed August 9, 1928. Serial No. 298,623.

This invention relates to lead compounds of the type which are used particularly for incorporating in certain classes of lubricants, and which are usually called "lead soaps".

5 In the usual method of manufacturing such "soaps" fatty oil consisting exclusively or largely of fatty acid glycerides is employed. Litharge (PbO) is mixed with the fatty oil and the whole is maintained at the high tem-  
10 perature with agitation until the litharge enters into combination.

Heretofore it has been the usual procedure to supply litharge to the extent of 3 molecular proportions to 2 molecular proportions 15 of the fatty oil, since the only lead soaps which are known in the literature are expressed by the formula  $(RCOO)_2Pb$ .

We have now discovered that soaps of this type are not produced to any considerable 20 extent by the interaction of litharge and fatty oils when processed as above described except to the extent that the oil contains free fatty acid. We have found that the fatty acid 25 glyceride is not saponified in the usual way, which is shown by the fact that substantially no glycerin or aldehydes are produced. The interaction between the glyceride and the litharge appears to be one of addition whereby 30 3 molecules of litharge become combined with a molecule of tri-glyceride to give a compound which we believe to be of the composition expressed by the empirical formula:  $(RCOO)_3C_5H_5.(PbO)_3$ . This fact has been established practically by analyzing lead

35 "soaps" produced from neutral fatty oils in the manner described above, such analysis showing that approximately one-half of the fatty oils has been converted into lead compounds of this type while the other one-half 40 remains substantially unchanged. Tests have shown that no glycerine is liberated and that no aldehydes are produced. Thus in the previous method of making lead soaps the 45 result is a mixture of lead compounds admixed with about one-half of the original fatty oil.

According to the present invention we 50 avoid the effectual waste of about one-half the fatty oils by increasing the quantity of

litharge substantially above the amount heretofore used, that is 3 molecular proportions of litharge to 2 molecular proportions of the tri-glyceride. We prefer to employ 3 molecular proportions of litharge to each molecular proportion of tri-glyceride although we may employ somewhat less litharge. Where the fatty oil contains free fatty acid we employ additional litharge for the purpose of converting the free acid into lead soaps of the type expressed in the first formula given above. When operating in this manner the compound becomes excessively stiff and effective agitation becomes difficult or practically impossible. Accordingly we 65 prefer to employ a suitable diluent, which may suitably be a hydrocarbon oil of relatively low viscosity and of such low volatility that it is not substantially evaporated during the manufacture of the lead compounds. In practice we prefer to employ a hydrocarbon oil of viscosity similar to that of the fatty oil employed and we prefer to use such oil in approximately the same amount by 70 volume as the fatty oil so that we produce a product which is similar in consistency and in lead compound content to the "lead soaps" heretofore produced. Such a product can be used as an ingredient in lubricants in the same manner as the product of the prior process without modification of 75 proportions.

It will be understood that the present invention is applicable to the production of lead compounds from various fatty oils. 80 Among those which have been used are dark-pressed fish oil, winter-bleached fish oil, mixed fish oils and soy bean oil.

In making the soap, the oil is diluted as indicated above, first heating to about 300° F. 85 and a small part of the litharge is added with efficient stirring. When the reaction begins, which is shown by the disappearance of the yellow color due to the presence of litharge, the litharge is added at a more rapid rate 90 and the whole is maintained at about the temperature indicated until the reaction is complete. This usually takes about one hour. Lower temperatures may be employed but the reaction is slower. The temperature 100

should not exceed about 325° F. for the best results.

The appropriate amount of lead oxide which should be employed with any suitable oil can readily be calculated from the free acidity of the oil and the saponification number.

The invention will more readily be understood from the following example: 45 pounds of dark pressed fish oil containing about 9% of free acid are mixed with about 22½ pounds of a light paraffin oil having a Saybolt viscosity of 95 to 100 sec. at 100° F. and a flash of about 340 to 350° F. and the mixture is heated in the manner described above. 32½ pounds of litharge are digested therein. The resulting product is analyzed and has the following composition.

|                  | Per cent |
|------------------|----------|
| 29 Lead compound | 75.42    |
| Neutral fat      | 1.60     |
| Paraffin oil     | 22.33    |
|                  | 99.35    |

25 For the purpose of comparison a "soap" is made from the same oil with the quantity of litharge ordinarily employed heretofore, that is, about one-half the quantity used in the preceding example. No diluent oil is employed. 75.2 pounds of the fish oil were caused to react with 27.5 pounds of litharge under the same conditions. The analysis of the resulting product is as follows:

|                  | Per cent |
|------------------|----------|
| 35 Lead compound | 66.46    |
| Neutral fat      | 32.94    |
|                  | 99.40    |

While the invention has been described with reference to the details of a specific example and specific conditions of operation, it is to be understood that the invention is not intended to be limited to such details or conditions, except in so far as included in the accompanying claims.

What we regard as new, and desire to secure by Letters Patent, is:

1. The method of making lead soap compounds which consists in causing litharge to react with fatty oils, said litharge being substantially in excess of 3 molecular proportions to 2 molecular proportions of the fatty oil.

2. The method of producing lead soap compounds which consists in causing reaction between litharge and fatty oils, the litharge being present to the extent of about 3 molecular proportions to each molecular proportion of fatty oil.

3. The method of producing lead soap compounds which consists in causing litharge to react upon fatty oil in the presence of a diluent, the litharge being present in amount substantially greater than 3 molecular proportions to 2 molecular proportions of fatty

oil, and the diluent being present in sufficient amount to maintain fluidity during the reaction.

4. The method of producing lead soap compounds which consists in causing reaction between litharge and fatty oil in the presence of a diluent, the litharge being present to the extent of about 3 molecular proportions for each molecular proportion of the fatty oil and the diluent being present in amount sufficient to maintain fluidity during the reaction.

5. The method of producing lead soap compounds which consists in causing reaction between litharge and fatty oil containing free acid, the litharge being present in amount substantially exceeding the litharge equivalent of the free acid and 3 molecular proportions of litharge to 2 molecular proportions of the unsaponified oil.

6. The method of producing lead soap compounds which consists in causing reaction between litharge and fatty oil containing free acid, in the presence of a diluent, the litharge being present in amount substantially exceeding the litharge equivalent of the free acid and 3 molecular proportions of litharge for each 2 molecular proportions of the unsaponified oil and the diluent being present in sufficient quantity to maintain fluidity during the reaction.

7. The method of producing lead soap compounds which consists in causing reaction between litharge and fatty oil containing free acid, the litharge being present in amount substantially equal to the litharge equivalent of the free acid and 3 molecular proportions of litharge to each molecular proportion of the unsaponified fatty oil.

8. The method of making lead soap compounds which consists in causing litharge to react with fatty oils at temperatures below 325° F., said litharge being substantially in excess of 3 molecular proportions to 2 molecular proportions of the fatty oil.

9. The method of producing lead soap compounds which consists in causing reaction between litharge and fatty oils at a temperature below 325° F., the litharge being present to the extent of about 3 molecular proportions to each molecular proportion of fatty oil.

10. The method of producing lead soap compounds which consists in causing litharge to react upon fatty oil in the presence of a hydrocarbon oil at a temperature below 325° F., the litharge being present in amount substantially greater than 3 molecular proportions to 2 molecular proportions of fatty oil, and the hydrocarbon oil being present in sufficient amount to maintain fluidity during the reaction.

11. The method of producing lead soap compounds which consists in causing litharge to react upon fatty oil in the presence of a hydrocarbon oil at a temperature below 325° F., the litharge being present to the ex-

tent of about 3 molecular proportions for each molecular proportion of the fatty oil, and the hydrocarbon oil being present in sufficient amount to maintain fluidity during the reaction.

5 12. The method of producing lead soap compounds which consists in causing litharge to react upon fatty oil in the presence of a light paraffin oil, the litharge being present 10 in amount substantially greater than 3 molecular proportions to 2 molecular proportions of fatty oil, and the diluent being present in sufficient amount to maintain fluidity during the reaction.

15 13. The method of producing lead soap compounds which consists in heating about 45 parts of fish oil with about 22½ parts of light paraffin oil to a temperature around 300° F., adding about 32½ parts of litharge 20 thereto and agitating until the litharge is digested therein.

14. A new composition of matter consisting of lead soap compounds of fatty oils, a hydrocarbon oil diluent, said composition 25 containing unchanged fatty oil in the proportion of less than 10% by weight of the lead soap compounds.

15. A new composition of matter comprising about 75% of compounds of lead oxide 30 with fatty oils, about 22% of a paraffin oil and less than 2% of unchanged fatty oil.

16. A new composition of matter consisting of lead soap compounds of fatty oils, and a hydrocarbon oil diluent, said composition 35 containing unchanged fatty oil in the proportion of less than 5% by weight of the lead soap compounds.

STERLING HENRY DIGGS.  
FRANK S. CAMPBELL.

40

45

50

55

60

65